

Aug. 18, 1936.

F. L. BOSQUI

2,051,433

PRODUCTION OF FERROCOPAL

Filed June 29, 1933



F. L. Bosqui  
INVENTOR

By: Marks & Clark  
A.H.S.

## UNITED STATES PATENT OFFICE

2,051,433

## PRODUCTION OF FERROCOPAL

Francis Lawrence Bosqui, N'Kana, Northern Rhodesia, assignor to Rhokana Corporation Limited, N'Kana, Northern Rhodesia

Application June 29, 1933, Serial No. 678,299

1 Claim. (Cl. 204—57)

In the metallurgical treatment of copper ores containing notable quantities of cobalt the latter metal may, by reduction of the copper slag, be obtained in the form of an alloy or mixture comprising cobalt, iron and copper. The object of the invention is to provide an electrolytic process whereby ferro-cobalt with a high degree of purity as regards copper may be obtained directly and cheaply from said alloy or mixture or similar material.

According to the invention, an alloy or mixture comprising iron, cobalt and copper is provided in which the copper does not exceed about 15% by weight. Said material is anodically corroded in an electrolytic cell, the electrolyte of which is substantially neutral, but is nevertheless on the acid side of neutrality. The free acid should be definitely below three grams per litre reckoned as sulphuric acid, otherwise copper would be deposited with the iron and cobalt; and in practice it is found desirable to maintain an amount of free acid ranging from one to two grams per litre, in order to keep the acidity of the electrolyte under control. During the operation of the electrolytic cell the copper content of the electrolyte is maintained at not more than about 0.05 gram per litre. Under these conditions cobalt and iron together are deposited as metal at the cathode whilst the copper content of the anode is for the most part left as sludge in the electrolytic cell.

The invention will be further described with reference to the accompanying diagrammatic drawing in which:

Figure I illustrates the production of ferro-cobalt in a single stage;

Figure II illustrates its production in several stages.

Referring to Figure I, 2 indicates an open electrolytic cell, that is a cell in which the anode and cathode are not separated by a diaphragm. The anode 3 is a casting of the raw material consisting of copper, iron and cobalt. The cathode 4 is a plate of material suitable for ferro-cobalt to plate onto such as rolled cobalt, iron, copper or stainless steel. 5 is a source of direct current such as to produce a current density of about 10 amperes per square foot of cathode area. The electrolyte 6 contains free acid, preferably sulphuric acid, to the extent of from one to two grams per litre.

Under these conditions the anode 3 is corroded; and, provided it does not contain an undue proportion of copper for instance not more than about fifteen per cent., there is de-

posited on the cathode a plating of commercially pure ferro-cobalt, that is ferro-cobalt containing not more than about 0.5 per cent. of copper.

The bulk of the copper appears as spongy copper and copper oxide. Some of this falls directly to the bottom of the cell. Some tends to collect on the anode surface and is brushed therefrom from time to time in order to prevent the anode surface from attaining too high a copper percentage, which would result in copper going in undue quantity into the solution.

A small amount of copper goes into solution and, unless controlled, it would build up in the electrolyte and deposit as metal on the cathode and thereby contaminate the ferro-cobalt. This, however, does not occur to any detrimental extent until the copper concentration of the electrolyte exceeds 0.05 gram per litre. The electrolyte may accordingly be treated to prevent the concentration from rising above that figure. This may be done by withdrawing a portion of the electrolyte, preferably continuously, treating such portion for the removal of its copper content and returning it to the cell. Such treatment conveniently consists in cementing the copper on to scrap iron or comminuted cobalt.

For this purpose the cell is provided with an outlet 7 from which the electrolyte can be continuously withdrawn at a rate controlled by the valve 8. It is then percolated through a mass 9 of material onto which it will cement such as scrap iron or comminuted cobalt or the ferro-cobalt product of the process. The latter is convenient owing to the physical form in which it often occurs, viz. as thin twisted and brittle scales, which are readily detached from the cathode and offer a large surface for the deposition of the copper.

The purified electrolyte is received at 10 and returned to the cell as indicated by 11.

The cement copper recovered at 9 as well as the copper sludge taken from the cell are in favourable physical and chemical condition for the recovery of the copper contents in pure form, as by smelting as indicated at 12.

The ferro-cobalt deposited at the cathodes is detached therefrom, melted under slightly reducing conditions and cast into shapes suitable for marketing.

When the copper content of the raw metal is high, say above fifteen per cent., the copper content of the deposited ferro-cobalt is correspondingly high. In order to obtain substantially pure

ferro-cobalt from raw metal high in copper, the operation is conducted in two or more stages as illustrated in Figure II. The impure ferro-cobalt obtained in the cell 2 is melted and cast into 5 anodes 3a which are corroded in a cell 2a under the same conditions as in cell 2. Strict adherence to the acid limitations mentioned above is not so essential in the preliminary purification stage or stages since, although an increase of 10 acidity would permit the deposition of copper to an extent which would not occur if the acid limits were adhered to, there is still a substantial reduction of the copper content relatively to the iron and cobalt content.

15 I claim:

The process of treating an alloy comprising iron cobalt and copper in which the copper content is substantially higher than 15% by weight, which consists in anodically corroding such ma-

terial in an electrolytic cell, the electrolyte of which contains acid in amount less than three grams per litre reckoned as sulphuric acid, thereby producing in the cell a cathode deposit of cobalt and iron containing less copper than the anode, repeating the step, if necessary, by using the cathode material of the earlier step as anode material in the later step until the material contains from trace to about 15% by weight of copper, then anodically corroding such material in 10 an electrolytic cell the electrolyte of which contains free acid less than three grams per litre reckoned as sulphuric acid, and the copper content of which does not exceed about 0.05 gram per litre, thereby anodically depositing iron and cobalt together substantially free from copper and causing the greater part of the remaining copper to deposit in the cell as sludge.

FRANCIS LAWRENCE BOSQUI.